

T. J. CURRY.

PROCESS FOR MAKING FORGED ANCHORS.  
APPLICATION FILED JUNE 11, 1919.

1,331,095.

Patented Feb. 17, 1920.

2 SHEETS—SHEET 1.



FIG. 1.



FIG. 2.



FIG. 3.



FIG. 4.



By

Thomas James Curry  
Attorney

T. J. CURRY,  
PROCESS FOR MAKING FORGED ANCHORS,  
APPLICATION FILED JUNE 11, 1919.

1,331,095.

Patented Feb. 17, 1920.

2 SHEETS—SHEET 2.



Inventor  
Thomas James Curry  
By  
John L. Curry  
attorney

# UNITED STATES PATENT OFFICE.

THOMAS JAMES CURRY, OF NETHERTON, NEAR DUDLEY, ENGLAND, ASSIGNOR TO N. HINGLEY & SONS, LIMITED, OF DUDLEY, ENGLAND.

## PROCESS FOR MAKING FORGED ANCHORS.

1,331,095.

Specification of Letters Patent.

Patented Feb. 17, 1920.

Application filed June 11, 1919. Serial No. 303,516.

To all whom it may concern:

Be it known that I, THOMAS JAMES CURRY, a subject of the King of England, and residing at Netherton, near Dudley, in the county 5 of Worcester, England, have invented Improvements in and Connected with Processes for Making Forged Anchors, of which the following is a specification.

This invention relates to a process for 10 making forged anchors from a single billet.

According to this invention, the anchor portion comprising the head proper, trippers, and arms or flukes are forged in one piece out of a single billet or body of malleable metal, generally steel, wherein the 15 tripper parts forged from the billet or block are extensions of the head portion on which the shank end is secured, and extend over the backs or outer edges of the arms or 20 flukes, which spring from points under and separated from the tripper parts and extend in a downwardly curved manner.

In the manufacture of a one-piece forged anchor, a hole is made in the center of the 25 billet or body, say of oblong form, adapted to constitute the aperture in which the head of the shank works; and on each side of this hole, and some distance from it, the billet at each side is shouldered down at a 30 certain point in the direction of length of the billet, and the parts outside the shouldered down portions constitute the parts of the forging which are to form the arms and flukes. At each angle at the shouldered 35 down parts, the metal of the billet or body is by hammering or pressing, and by suitable tools, recessed down at each outside portion on each side, into comparatively thin plates, which parts are to form the trippers of the 40 anchor.

On the outer side of the forging so far made, the portions which are to form the arms and flukes are set down to the depth or thickness of the trippers; and they are 45 forged or pressed down all along on this side, the other side of the arm parts remaining flush or practically so with the inside face of the head portion proper which surrounds the hole.

Beyond the trippers the edges of the arms 50 are forged or pressed down, and tapered to the tips, and at the end of these tapered parts, part of the metal is hammered or pressed out by suitable tools, to form comparatively thin plates on each side which

are to constitute the flukes or palms on the ends of the arms.

The forging is now severed between the tripper portions of the head, and the outer parts of the arms by sawing, milling, slotting or otherwise, up to the head portion proper which surrounds the aperture, which may be of the full depth of the original billet or body; and each arm at the shoulder is heated by a separate fire or heating medium, while the head itself is kept cool, and a mandrel or part is passed through the aperture in the head, and the head is held in position thereby on a suitable holding bed or the like; and then while the arm parts 60 are hot, they are bent around, say by pulling up by a crane or otherwise, over a shaped former, which is held say by the mandrel, and which is on the outside of the usual curvature of the inside of the arms. 65

This anchor head and fluke portion and its process of manufacture or forging is illustrated by the annexed drawings, which 70 illustrate the various conditions of form produced by the several operations performed upon it, these operations being done preferably in the order of the numerals of the figures.

In the drawings the Figures 1 to 11 represent the successive and various steps in carrying out the method of forming an anchor. 80

Fig. 1 shows the billet or block of metal with the first operation formed on it, namely, the swaging of the shank hole 1, which will be effected by suitable tools used 90 for such forging operations.

Fig. 2 shows the billet or body after the next operation, which consists in shouldering down the ends of the billet front points which are to form the extremity of the head 95 of the anchor, that is the edges of the tripper portions of same; the metal displaced by this action being transferred in length of the parts 2 which are to form the arms or flukes, and their palms or tips. 100

Fig. 3 shows the metal after the next operation has been performed, which consists in recessing down the corners of the forging between the roots of the arm members 2, and the head portion 3. The metal thus pressed down and displaced takes the form of the extended portions 4 at each corner of the head. This operation may be made by V setting or other suitable tools; and these parts 4 form the tripper parts of the anchor. 105 110

As the metal pressed out by this latter operation may extend in a rounded manner, as indicated by the full lines in the figure, the outer edges of these parts will be cut off 5 along the line 5\*, so as to make the edges of the trippers square, but still projecting out beyond the sides of the head portion proper 3; as seen in the next figure.

In the next operation the elongation of the 10 arms or flukes 2 is effected, this being shown in Fig. 4. In this operation, from the inner angle of the recesses on the underside of the tripper parts 4, the arm portions 2 are forged downward in a tapered manner 15 shown in this figure, and also they are set down as indicated in Fig. 5 at the back side, so that the upper side of the arms will then be in the same plane as the undersides of the trippers. The palms or tip portions 5 may 20 then be forged to the form required.

The next operation is that of severing the tripper parts 4 from the arms or flukes 2 by sawing or milling; the severing cut being marked 6 in Fig. 6.

25 The arms are then heated by separate applications of heat as above described, on each side of the head proper 3 which is kept cool as stated; and then the main final operation is the bending of the arm portions 2 around into the shape required, of which Fig. 7 shows a suitable one.

Thus by this process and method, the whole head portion of the anchor, namely, the head proper 3, trippers 4, and arms or 35 flukes 2 with their palms or tips 5, are forged and made by a simple sequence of forging operations from a solid plain billet or body of malleable metal.

With regard to the actual sequence of operations employed in the manufacture of the anchor, it is to be stated that this may be varied somewhat—as will be understood by those skilled in the art—and some of the operations transposed, without departing 45 from the substance of the invention.

With regard to the securing of the shank head in the anchor head 3 proper, two known modes of connection are shown in Figs. 8 and 9, and Figs. 10 and 11, respectively.

50 In the case shown in Fig. 8 and 9, the connection of shank 10 and head 3 is by a pin 8 passing through the tops or roots of the flukes or arms 2, and the lower portion of the head 3; the pin being secured in po-

sition by nuts 9 screwing on to the ends of 55 the same, and the nuts lying in cut out recesses, in the arm root portions.

In the case shown in Figs. 10 and 11, the pin 8 in the head of the shank 10 lies in recesses at each side of the hole 1, extending 60 down from the outer face of the head; and above the ends of the pin 8, caps 11, formed on the ends of vertical bolts 12, are fitted; and they are secured in position by nuts 13 screwing on the bolts on the inner side 65 of the head 3.

It will be seen in the anchors shown in Figs. 8 to 11, the arms or flukes 2 taper from wide roots next the head, to more or less thin tips; but they may be of any suitable 70 shape. It will also be seen in these figures, the angles of the lower part of the head 3 at each side of the aperture 1 (which is of the usual form used in this kind of anchor) are rounded; but they may be rectangular or of 75 any required shape.

What is claimed is:—

1. The process of making a forged anchor from a single billet, consisting in forging the ends of same to produce extensions to 80 form arms of less width than the original billet, forging and indenting the metal at the angles between the extensions and the remaining portion of the original billet to reduce the thickness of said metal, the metal 85 at these points to form tripper parts on each side of the arms, and subsequently separating said parts from the arms.

2. The process of making a forged anchor from a single billet, consisting in forging 90 the ends of same to produce extensions to form arms of less width than the original billet, forging and indenting the metal at the angles between the extensions and the remaining portion of the original billet to 95 reduce the thickness of said metal, the metal at these points to form tripper parts on each side of the arms, separating said part from the arms, and subsequently bending the arms to further separate the same from the trip- 100 per parts.

In testimony whereof I have signed my name to this specification in the presence of two subscribing witnesses.

THOMAS JAMES CURRY.

Witnesses:

JAMES L. GRAINGER,  
SYDNEY G. DAVIES.